



US009863094B2

(12) **United States Patent**  
**Pang et al.**

(10) **Patent No.:** **US 9,863,094 B2**  
(45) **Date of Patent:** **\*Jan. 9, 2018**

(54) **PRINTABLE COMPOSTABLE PAPERBOARD**(71) Applicant: **WestRock MWV, LLC**, Norcross, GA (US)(72) Inventors: **Jiebin Pang**, Glen Allen, VA (US); **Natasha G. Melton**, Richmond, VA (US); **Steven Parker**, Raleigh, NC (US)(73) Assignee: **WestRock MWV, LLC**, Norcross, GA (US)

(\* ) Notice: Subject to any disclaimer, the term of this patent is extended or adjusted under 35 U.S.C. 154(b) by 0 days.

This patent is subject to a terminal disclaimer.

(21) Appl. No.: **15/258,181**(22) Filed: **Sep. 7, 2016**(65) **Prior Publication Data**

US 2017/0002517 A1 Jan. 5, 2017

**Related U.S. Application Data**

(63) Continuation-in-part of application No. 15/230,896, filed on Aug. 8, 2016, now Pat. No. 9,670,621, which is a continuation-in-part of application No. 15/017,735, filed on Feb. 8, 2016, now Pat. No. 9,771,688.

(60) Provisional application No. 62/372,403, filed on Aug. 9, 2016, provisional application No. 62/164,128, filed on May 20, 2015, provisional application No. 62/114,716, filed on Feb. 11, 2015.

(51) **Int. Cl.**

**D21H 21/14** (2006.01)  
**D21H 19/40** (2006.01)  
**D21H 19/38** (2006.01)  
**D21H 27/22** (2006.01)  
**D21H 27/10** (2006.01)  
**D21H 23/48** (2006.01)  
**D21H 23/50** (2006.01)  
**D21H 23/56** (2006.01)  
**D21H 23/72** (2006.01)  
**D21H 19/44** (2006.01)  
**D21H 19/58** (2006.01)  
**D21H 19/60** (2006.01)  
**D21H 19/82** (2006.01)  
**D21H 21/16** (2006.01)  
**D21H 23/32** (2006.01)  
**D21H 23/34** (2006.01)

(52) **U.S. Cl.**

CPC ..... **D21H 21/14** (2013.01); **D21H 19/38** (2013.01); **D21H 19/385** (2013.01); **D21H 19/40** (2013.01); **D21H 19/44** (2013.01); **D21H 19/58** (2013.01); **D21H 19/60** (2013.01); **D21H 19/82** (2013.01); **D21H 21/16** (2013.01); **D21H 23/32** (2013.01); **D21H 23/34** (2013.01); **D21H 23/48** (2013.01); **D21H**

**23/50** (2013.01); **D21H 23/56** (2013.01); **D21H 23/72** (2013.01); **D21H 27/10** (2013.01); **D21H 27/22** (2013.01)

(58) **Field of Classification Search**

CPC ..... D21H 21/14; D21H 19/38; D21H 19/385; D21H 19/40; D21H 19/44; D21H 19/58; D21H 19/60; D21H 19/82; D21H 19/822; D21H 21/16; D21H 23/32; D21H 23/34; D21H 23/48; D21H 23/50; D21H 23/56; D21H 23/72; D21H 27/10; D21H 27/22

USPC ..... 428/537.5

See application file for complete search history.

(56) **References Cited**

## U.S. PATENT DOCUMENTS

5,776,619 A \* 7/1998 Shanton ..... A47G 19/03 427/326  
5,981,011 A \* 11/1999 Overcash ..... D21H 19/16 428/34.2  
6,074,733 A \* 6/2000 Falat ..... B65D 65/42 428/219  
6,740,373 B1 \* 5/2004 Swoboda ..... B32B 29/06 229/5.81  
7,404,999 B2 7/2008 Wilhoit et al.  
7,833,915 B2 11/2010 Propst  
8,597,733 B2 12/2013 Vonfelden  
2004/0121080 A1 \* 6/2004 Urscheler ..... B05D 1/305 427/420  
2011/0262745 A1 10/2011 Ronka  
2013/0330527 A1 12/2013 Hartmann et al.  
2014/0113152 A1 4/2014 Zischka et al.  
2014/0120277 A1 5/2014 Vonfelden  
2014/0272352 A1 9/2014 Tilton

## FOREIGN PATENT DOCUMENTS

EP 0718437 A1 9/2003  
EP 1940561 A1 7/2008  
EP 2719825 A1 4/2014  
WO WO2006/007239 \* 1/2006  
(Continued)

## OTHER PUBLICATIONS

International Search Report and Written Opinion for PCT/US2016/017463, dated May 10, 2016.

Primary Examiner — Leszek Kiliman

(74) Attorney, Agent, or Firm — WestRock Intellectual Property Group

(57) **ABSTRACT**

A coated paperboard is disclosed which includes a barrier coating containing substantially no fluoroochemical or wax, exhibiting good resistance to oil and grease, no tendency toward blocking, the coated paperboard being fully repulpable as well as compostable. The coated paperboard may further have a printable coating on a surface opposite from the barrier coating.

(56)

**References Cited**

FOREIGN PATENT DOCUMENTS

|    |               |    |         |
|----|---------------|----|---------|
| WO | WO2006007239  | A2 | 1/2006  |
| WO | WO2009142731  | A1 | 11/2009 |
| WO | WO2010042162  | A1 | 4/2010  |
| WO | WO2013/189550 | *  | 12/2013 |
| WO | WO2013189550  | A1 | 12/2013 |
| WO | WO2014/006269 | *  | 1/2014  |
| WO | WO2014006269  | A1 | 1/2014  |
| WO | WO2015003275  | A1 | 1/2015  |

\* cited by examiner

**FIG. 1**

**FIG. 2**

**FIG. 3**

**FIG. 4**



FIG. 6



FIG. 7



## PRINTABLE COMPOSTABLE PAPERBOARD

## REFERENCE TO RELATED APPLICATIONS

This application is a continuation in part of U.S. application Ser. No. 15/230,896 filed on Aug. 8, 2016, which is a continuation in part of U.S. application Ser. No. 15/017,735 filed on Feb. 8, 2016, which claims the benefit of priority under 35 U.S.C. §119(e) of U.S. provisional application Ser. No. 62/114,716 filed on Feb. 11, 2015, and Ser. No. 62/164,128 filed on May 20, 2015, all of which are incorporated herein by reference in their respective entireties. This application also claims the benefit of priority under 35 U.S.C. §119(e) of U.S. provisional application Ser. No. 62/372,403 filed on Aug. 9, 2016 which is incorporated herein by reference in its entirety.

## BACKGROUND OF THE INVENTION

## Field of Invention

This disclosure relates to paperboard substrates having oil and grease resistance, yet with full recyclability and without having a tendency toward blocking, and furthermore being compostable.

## Description of the Related Art

Sustainable packages using renewable, recyclable, and/or compostable materials are increasingly and strongly desired for food service and food packaging. Paper or paperboard itself is one of the most sustainable materials for packaging applications; however, paper or paperboard is often coated or laminated with barrier materials to fulfill the requirements of packaging. These additional barrier coatings or films often make the finished packages no longer repulpable or compostable. For example, widely used polyethylene coated paperboard is neither compostable nor recyclable under typical conditions. Polylactide coated paperboard can be compostable under industrial conditions, but it is not recyclable.

Oil and grease resistance is one of the top needs for paperboard packages in food and food service industries. Several technologies including specialty chemical (wax, fluorochemicals, starch, polyvinyl alcohol (PVOH), sodium alginate, etc.) treatment, polymer extrusion coating (polyethylene, etc.) have been employed to provide oil and grease resistance of paperboard packaging. However, the paper or paperboard treated with wax or coated with polyethylene, which is currently used in oil and grease resistant packaging, has difficulties in repulping and is not as easily recyclable as conventional paper or paperboard. Paper or paperboard treated with specialty chemicals such as fluorochemicals has potential health, safety and environmental concerns, and scientists have called for a stop to non-essential use of fluorochemicals in common consumer products including packaging materials.

There is a need for oil and grease resistant paperboard that is recyclable, compostable, low cost, and without environmental or safety concerns. Aqueous coating is one of the promising solutions to achieve these goals. However, blocking (the tendency of layers in a roll of paperboard to stick to one another) is a challenging technical hurdle in production and converting processes for aqueous barrier coated paperboard, and blocking is also a major technical hurdle for on-machine application of aqueous barrier coatings. Furthermore, most aqueous barrier coatings are not fully repulpable. Commonly-assigned U.S. application Ser. No. 15/017,735 which is incorporated herein by reference, addresses these problems. However, it is further desired to

have a paperboard that is compostable. The ASTM D6868-11 Standard Specification for compostability of paper or paperboard requires any non-biodegradable organic constituent to be <1% of the dry weight of the finished product, and the total portion of organic constituents that are not biodegradable cannot exceed 5% of the total weight. Most conventional or commercially available aqueous barrier coatings use high to pure synthetic polymer binder level, which makes it extremely challenging to meet this <1% non-biodegradable composition requirement for the ASTM compostability standard, while achieving the barrier performance required by the package.

## SUMMARY OF THE INVENTION

In the present work, certain inventive coatings that have barrier properties have achieved the ASTM compostability standard, at least for paperboard that is 12 caliper (0.012") or higher. With lower caliper paperboards, the coating(s) typically contribute a larger share of the total weight, with the result that the non-biodegradable organic constituent in the coatings becomes more than 1% of such lower-caliper paperboard.

The general purpose of the invention is to coat the 'barrier' side of a paperboard with at least one layer of aqueous coating containing a renewable natural material (modified starch) and a specialty synthetic binder, resulting in the coated oil and grease resistant paperboard (i.e., 12 pt caliper and above) meeting the <1% non-biodegradable composition requirement for the compostability standard. The coating can either be applied on a paper machine or by an off-line coater, and can be applied in two coating steps (or two passes) for further enhanced barrier properties. Paperboard coated according to the invention provides resistance to oil and grease, does not have any tendency to block, is compliant to safety and environmental regulations, is fully repulpable, is compostable, and can be produced at a low cost.

In one embodiment a coated paperboard is disclosed which includes a paperboard substrate having a first side and a second side; a first coating in contact with the first side, the first coating having a coat weight from 5 to 12 lbs per 3000 ft<sup>2</sup> and comprising binder and pigment, the first coating containing substantially no fluorochemical or wax; a second coating in contact with the second side, wherein the second coating is a printable coating; wherein the coated paperboard has a caliper of at least 0.010"; wherein the coated paperboard provides barrier properties to at least one of oil, grease, and moisture; wherein the coated paperboard is compostable according to the ASTM D6868-11 standard for compostability; and wherein the coated paperboard is at least 99% repulpable.

In one embodiment a method of treating paperboard is disclosed, the method including providing a paperboard substrate having a first side and a second side; applying to the first side a coating comprising binder and pigment, and containing substantially no fluorochemical or wax; applying to the second side a printable coating; wherein the binder comprises starch; wherein the treated paperboard has a caliper of at least 0.010"; wherein the treated paperboard is compostable according to the ASTM D6868-11 standard for compostability; wherein the treated paperboard has a 3M kit test value of at least 3; and wherein the treated paperboard is repulpable to the extent that after repulping the percentage accepts is at least 99%.

In one embodiment, a coated paperboard is disclosed which includes a paperboard substrate; a base coating in

contact with the paperboard substrate, the base coating having a coat weight from 6 to 10 lbs per 3000 ft<sup>2</sup> and comprising binder and pigment; a top coating in contact with the base coating, the top coating having a coat weight from 4 to 7 lbs per 3000 ft<sup>2</sup> and comprising binder and pigment; wherein the coated paperboard has a caliper of at least 0.010"; and wherein the coated paperboard is compostable according to the ASTM D6868-11 standard for compostability.

#### BRIEF DESCRIPTION OF THE DRAWINGS

FIG. 1 illustrates a method for producing a base stock on a paperboard machine;

FIG. 2 illustrates a method for treating the base stock from FIG. 1 by applying coatings to both sides on a paperboard machine;

FIG. 3 illustrates a method for treating the base stock from FIG. 1 by applying coatings to one side on a paperboard machine;

FIG. 4 illustrates a method for treating the base stock from FIG. 1 by applying coatings to one side on an off-machine coater;

FIG. 5 illustrates a device for measuring blocking of paperboard;

FIG. 6 is a graph of oil/grease resistance (3M kit level) vs. coat weight for several coatings; and

FIG. 7 is a graph of oil resistance (Cobb) vs. coat weight for several coatings.

#### DETAILED DESCRIPTION OF THE INVENTION

FIG. 1 and FIG. 2 illustrate an exemplary on-paper machine method for coating a paperboard web with one or more layers of aqueous coating. A forming wire 110 in the form of an endless belt passes over a breast roll 115 that rotates proximate to a headbox 120. The headbox provides a fiber slurry in water with a fairly low consistency (for example, about 0.5% solids) that passes onto the moving forming wire 110. During a first distance 230 water drains from the slurry and through the forming wire 110, forming a web 300 of wet fibers. The slurry during distance 130 may yet have a wet appearance as there is free water on its surface. At some point as drainage continues the free water may disappear from the surface, and over distance 231, water may continue to drain although the surface appears free from water.

Eventually the web is carried by a transfer felt or press felt through one or more pressing devices such as press rolls 130 that help to further dewatering the web, usually with the application of pressure, vacuum, and sometimes heat. After pressing, the still relatively wet web 300 is dried, for example using dryer or drying sections 401, 402 to produce a dry web ("raw stock") 310 which may then be run through a size press 510 that applies a surface sizing to produce a sized "base stock" 320 which may then be run through additional dryer sections 403 and (on FIG. 2) smoothing steps such as calendar 520.

The base stock 320 may then be run through one or more coaters. For example, coater 530 may apply a first coat ("BC") to a first side ("C1") of the web, and the first coat may be dried in one or more dryer sections 404. Coater 540 may apply a second coat ("TC") to the first side of the web, and the second coat may be dried in one or more dryer sections 405.

If the web is to be coated on two sides, coater 550 may apply a first coat to the second side ("C2") of the web, and this coat may be dried in one or more dryer sections 406. Coater 560 may apply a second coat to the second side of the web, and this coat may be dried in one or more dryer sections 407. The order of coaters 540, 550 may be swapped, so that both sides C1 and C2 are first given a first coat, and then one side or both sides are given a second coat. In some instances only one side will be coated as shown in FIG. 3, or only a first coat may be applied. In some instances a third coat may be applied to one side.

Instead of applying coating by on-machine coaters as shown in FIGS. 2 and 3, coating may be applied by an off-machine coater as shown in FIG. 4. In such cases, the paperboard having been produced on the paper machine and wound onto reel 572 may then be transported (as a reel or as smaller rolls) to an off machine coater 600, where the paperboard is unwound from reel 572, given a first coating by coater 610, dried in dryer(s) 601, given an optional second coating by coater 620, dried in dryer(s) 602, optionally given further treatment (such as gloss calendaring) and then wound onto reel 573. An off machine coater could instead apply a single coat to one side of the paperboard, or could apply a single coat to each side, or could apply more than one coat to either or both sides. Alternately some coating may be done on the paper machine, with additional coating done on an off-machine coater.

Various types of coating devices may be used. The coaters illustrated in FIGS. 2-4 are devices where a coating is held in a pan, transferred by a roll to the lower surface of the web (which may be either the first side or the second side depending on the web path), and then the excess coating scraped off by a blade as the web wraps partially around a backing roll. However other coater types may be used instead, including but not limited to curtain coater, air knife coater, rod coater, film coater, short-dwell coater, spray coater, and metering film size press.

The particular materials used in the coatings may be selected according to the desired properties of the finished paperboard. For example one side e.g. C1 may be given coating(s) that provide desired printability, while the other side e.g. C2 may be given barrier coating(s) that provide oil and grease resistance (OGR). The printability coating may be applied before the OGR coating, or, the OGR coating may be applied before the printability coating.

Following the coaters, there may be additional equipment for further processing such as additional smoothening, for example gloss calendaring. Finally, the web is tightly wound onto a reel 570.

The general process of papermaking and coating having been outlined at a high level in the preceding description and with FIGS. 1-4, we now turn to the coatings of the present invention. Typical aqueous barrier coatings often use specialty polymer(s), wax, and/or a higher polymer binder level (compared to conventional print coatings). These coatings can cause problems with repulpability of the coated paperboard because the coatings are usually difficult to breakdown to acceptable size or tend to form 'stickies' in paperboard making with the recycled fibers. Due to the high content of synthetic polymer binder in the coating, it is extremely challenging for each of the individual organic components in the coating to meet the <1% non-biodegradable composition requirement of the ASTM D6868-11 compostability standard.

Furthermore, many barrier coatings give paperboard a tendency to 'block' (the layers stick together) either in the reel 570, 571, 572, 573 or after it is rewound into rolls.

Particularly in the reel 570, there may be residual heat from the dryers, which may dissipate quite slowly because of the large mass of the reel. Higher temperatures may increase the tendency toward blocking.

It is known that paperboard coated with conventional printability coatings usually does not block, and usually is fully repulpable. It would be advantageous if non-blocking and fully repulpable coatings also provided at least some degree of barrier properties. However, conventional printability coatings do not provide satisfactory barrier properties. Their formulations have relatively low levels of binder so as to absorb rather than repel fluid (printing ink, for example).

Binder amounts in conventional printability coatings can range from 15-25 parts per 100 parts of pigment by weight for base coatings, and 10-20 parts per 100 parts pigment by weight for top coatings. Printing grades would tend to be in the lower half of these ranges. Limiting the binder amount in the top coating may allow printing inks or adhesives to absorb readily into the printability coating. Simply increasing the binder to improve barrier properties eventually interferes with printability and causes additional problems, including blocking and repulpability problems.

Similar blocking and repulpability problems exist with many aqueous barrier coatings that use specialty polymer(s) and/or a higher polymer binder level (compared to printability coatings), with the deleterious effect that the coated paperboard is not completely recyclable and tends to block at elevated temperature or pressure.

In contrast, the inventive coatings disclosed in the present application provide easy repulping, meet the composition requirement for the ASTM compostability standard, do not block at elevated temperature and pressure, and show good barrier properties, while using conventional pigments and synthetic and natural binders that are low-cost and readily available as coating materials for the paper or paperboard industry.

Conventional pigments are used in the present invention and may include, but are not limited to, kaolin clay, calcium carbonate, etc. Pigments used in the examples herein are given the following 'shorthand' designations:

"Clay-1" kaolin clay, for example, a No. 1 ultrafine clay  
"Clay-2" platy clay with high aspect ratio

"CaCO<sub>3</sub>-1" coarse ground calcium carbonate (particle size 60%<2 micron)

"CaCO<sub>3</sub>-2" fine ground calcium carbonate (particle size 90%<2 micron)

Synthetic polymer binders may include, but are not limited to, styrene acrylate copolymer (SA), polyvinyl acetate (PVAc), and styrene-butadiene copolymer (SB), etc. Natural binders may include, but are not limited to, starch, alginate, protein, etc. Conventional styrene acrylate binder (SA, PHOPLEX® C-340, available from Dow Chemical Company), acrylic polymer binder (Basonal® X400AL, available from BASF Corporation), starch binder (Pen-Cote® D UHV, available from Ingredion Incorporated), or a blend of Pen-Cote® D with SA or Basonal®, are used in examples described herein. Benefits of using Pen-Cote® D include its being directly dispersible into the formulation, increasing the coating formulation solids, and possibly being able to eliminate other thickeners. The choice of binder in the examples is not meant to be limiting in any way.

Coatings including control coatings in the present invention were prepared according to the formulations shown in Table 1, which provides a list of major constituents in dry parts of the aqueous coating (C—Control, CF—Compostable Formulation) formulations used to achieve the oil

and grease resistance, and to meet the composition requirement for the ASTM compostability standard, without blocking or repulpability problems. The test results are shown in Tables 3 and 4.

Substantially no fluorochemical was used in the coatings. By "substantially no fluorochemical" is meant that fluorochemicals were not deliberately utilized, and that any amount present would have been at most trace amounts. Although fluorochemicals can be excluded in lab experiments, trace amounts of such materials might be present in some paper machine systems due to making various grades of product, or might be introduced into a papermaking system through recycling processes. Likewise substantially no wax was used in the coatings.

The total binder to pigment ratio (parts of binder, by weight, to 100 parts of pigment) of the formulations shown in Table 1 ranges from 30 to 35. This is more than the binder to pigment ratio for typical printability coatings (where rapid absorption of ink is desired) and less than the binder to pigment ratio of typical barrier coatings. Thus it appears that an effective binder to pigment ratio may be from about 25 to about 40 parts binder per 100 parts pigment (by weight), or from 30 to 35 parts binder per 100 parts pigment. However, perhaps acceptable results (good 3M kit test, no blocking, and good repulpability) might be achieved with a slightly greater range. Blending starch (such as Pen-Cote® D), a natural biodegradable material, into the formulation helps meet the <1% non-biodegradable composition requirement for the ASTM compostability standard while maintaining the barrier performance. The Pen-Cote® D starch was added at up to 5 parts in the final formulations.

Paperboard samples were made using solid bleached sulphate (SBS) substrate with a caliper of 18 pt (0.018"). The samples were coated on one side (herein termed the "barrier side") using a pilot blade coater with a one-layer coating. The pilot results are expected to be representative of results that might be achieved on a production paper machine or a production off-machine coater.

The oil and grease resistance (OGR) of the samples was measured on the 'barrier side' by the 3M kit test (TAPPI Standard T559 cm-02). With this test, ratings are from 1 (the least resistance to oil and grease) to 12 (excellent resistance to oil and grease penetration). The results here gave 3M kit levels between 1 to 6 (see Table 3). The higher values were obtained with the higher coat weights for each specific formulation. Most interestingly, it is found that Basonal® binder itself (C2 formulation) performs better on 3M kit level than SA binder (C1 formulation) at comparable coat weights (see Table 3); furthermore, blending Pen-Cote® D starch with Basonal® (CF1-3) maintains the performance on 3M kit level as using Basonal® itself at comparable or slightly higher coat weight, while meeting the <1% non-biodegradable composition requirement for the ASTM compostability standard. Especially, a 3M kit level of 4-5 (suitable for most food service packages) is achieved while meeting the compostability standard.

In addition to 3M kit test, oil absorptiveness (oil Cobb) was used to quantify and compare the OGR performance (oil and grease resistance), which measures the mass of oil absorbed in a specific time, e.g., 30 minutes, by 1 square meter of coated paperboard. For each condition tested, the sample was cut to provide two pieces each 6 inch×6 inch square. Each square sample was weighed just before the test. Then a 4 inch×4 inch (area of 16 square inches or 0.0103 square meters) square of blotting paper saturated with peanut oil was put on the center of the test specimen (barrier side) and pressed gently to make sure the full area of oily

blotting paper was contacting the coated surface. After 30-minutes as monitored by a stop watch, the oily blotting paper was gently removed using tweezers, and the excess amount of oil was wiped off from the coated surface using paper wipes (Kimwipes™). Then the test specimen was weighed again. The weight difference in grams before and after testing divided by the test area of 0.0103 square meters gave the oil Cobb value in grams/square meter.

As the oil Cobb results shown in Table 3, all the formulations (CF1-4) containing Basonal® and Pen-Cote® D starch showed similar or improved (lower) oil Cobb value compared to both control formulations (C1 or C2), while all of them met the ASTM compostability standard. This confirmed the 3M kit results; and most interestingly, although CF4 at a coat weight 11.3 lb/3 msf showed a 3M kit level of 3.8, it performed very well on actual oil holdout showing an oil Cobb of 4.9 gsm in 30 minutes (Table 3)

Moisture resistance of the coatings was evaluated by WVTR (water vapor transmission rate at 38° C. and 90% relative humidity; TAPPI Standard T464 OM-12) and water Cobb (TAPPI Standard T441 om-04). All the formulations (CF1-4, Table 3) containing Basonal® and Pen-Cote® D starch showed similar water Cobb and WVTR values compared to both control formulations (C1 or C2), while all of them met the ASTM compostability standard.

The blocking behaviour of the samples was tested by evaluating the adhesion between the barrier coated side and the other uncoated side. A simplified illustration of the blocking test is shown in FIG. 5. The paperboard was cut into 2"×2" square samples. Several duplicates were tested for each condition, with each duplicate evaluating the blocking between a pair of samples 752, 754. (For example, if four duplicates were test, four pairs—eight pieces—would be used.) Each pair was positioned with the ‘barrier-coated’ side of one piece 752 contacting the uncoated side of the other piece 754. The pairs were placed into a stack 750 with a spacer 756 between adjacent pairs, the spacer being foil, release paper, or even copy paper. The entire sample stack was placed into the test device 700 illustrated in FIG. 5.

The test device 700 includes a frame 710. An adjustment knob 712 is attached to a screw 714 which is threaded through the frame top 716. The lower end of screw 714 is attached to a plate 718 which bears upon a heavy coil spring 720. The lower end of the spring 720 bears upon a plate 722 whose lower surface 724 has an area of one square inch. A scale 726 enables the user to read the applied force (which is equal to the pressure applied to the stack of samples through the one-square-inch lower surface 724).

The stack 750 of samples is placed between lower surface 724 and the frame bottom 728. The knob 712 is tightened until the scale 726 reads the desired force of 100 lbf (100 psi applied to the samples). The entire device 700 including samples is then placed in an oven at 50° C. for 24 hours. The device 700 is then removed from the test environment and cooled to room temperature. The pressure is then released and the samples removed from the device.

The samples were evaluated for tackiness and blocking by separating each pair of paperboard sheets. The results were reported as shown in Table 2, with a 0 rating indicating no tendency to blocking.

Blocking damage is visible as fiber tear, which if present usually occurs with fibers pulling up from the non-barrier surface of samples 754. If the non-barrier surface was coated with a print coating, then blocking might also be evinced by damage to the print coating.

For example, in as symbolically depicted in FIG. 5, samples 752(0)/754(0) might be representative of a “0” blocking (no blocking). The circular shape in the samples indicates an approximate area that was under pressure, for instance about one square inch of the overall sample. Samples 752(3)/754(3) might be representative of a “3” blocking rating, with up to 25% fiber tear in the area that was under pressure, particularly in the uncoated surface of sample 754(3). Samples 752(4)/754(4) might be representative of a “4” blocking rating with more than 25% fiber tear, particularly in the uncoated surface of sample 754(4). The depictions in FIG. 5 are only meant to approximately suggest the percent damage to such test samples, rather than showing a realistic appearance of the samples.

Repulpability was tested using an AMC Maelstrom repulper. 110 grams of coated paperboard, cut into 1"×1" squares, was added to the repulper containing 2895 grams of water (pH of 6.5±0.5, 50° C.), soaked for 15 minutes, and then repulped for 30 minutes. 300 mL of the repulped slurry was then screened through a Vibrating Flat Screen (0.006" slot size). Rejects (caught by the screen) and fiber accepts were collected, dried and weighed. The percentage of accepts was calculated based on the weights of accepts and rejects, with 100% being complete repulpability.

As an example of poor repulpability, SBS paperboard coated with low density polyethylene (LDPE) at a coat weight of 7-11 lbs per 3000 ft<sup>2</sup> was tested and gave fiber accepts in a range of 91 to 97%. (A fiber accepts percentage close to 100% is desired). Paperboard coated with polyethylene not easily repulpable and recyclable.

Various coating formulations shown in Table 1 were applied as single layers onto a paperboard substrate, using a range of coat weights, and the results are shown in Table 3 including repulpability and compostability. All of the samples were fully repulpable. As for compostability, as seen in the first two columns of Table 3, paperboard C1 with coating using a pure styrene acrylate (SA) binder did not meet the definition of compostable at coat weights of 9-10 pounds. Furthermore these C1 samples blocked slightly, whereas the other samples did not. The next two columns show that paperboard C2 with coating using a Basonal® X 400 AL binder (made by BASF Corporation) met the definition of compostability at a coat weight of 8 pounds, but not at a coat weight of 9 pounds. The last four columns (paperboard CF1, CF2, CF3, CF4) are for coatings blending the

Basonal® binder with Pen-Cote® D, a modified starch made by Ingredion Incorporated. These paperboards all meet the compostability definition.

Also included in Table 3 are measurements of Gloss, Brightness, Whiteness, and L-a-b Color. Gloss was measured on a Technidyne Model T 480A Glossmeter according to TAPPI standard T480. (GE) Brightness was measured on a Technidyne Brightimeter Micro S-5 according to TAPPI standard T452. (CIE) Whiteness was measured the Technidyne Brightimeter Micro S-5 according to TAPPI standard T562. L-a-b color was measured on the Technidyne Brightimeter Micro S-5 according to TAPPI standard T524. Using Basonal® binder or a blend of Basonal® binder with Pen-Cote® D starch showed similar or slightly higher gloss of the coating than using SA binder, but with slightly lower brightness and whiteness and slightly higher b-color value. Barrier properties are the focus of the inventive coatings, however, if there is a need to adjust the color or shade, food contact compliant dyes can be used in the formulations.

Another experiment was done by applying the CF3 formulation in two passes on a blade coater, with the first layer coat weight of 5.7 lb/3 msf and the second layer coat weight of 3.0 lb/3 msf, resulting a total coat weight of only 8.7 lb/3 msf, which met the composition requirement for compostability standard and showed a 3M kit value of 6.0. As shown from Table 4, a kit level of 5.2 was obtained when a single layer of CF3 was applied with a higher coat weight of 9.7 lb/3 msf. These results demonstrated that enhanced barrier properties can be obtained with two passes of the barrier formulations.

The Basonal® X 400 AL binder made by BASF Corporation contains about 30% natural polymer component. A natural polymer component refers to one grown and found in nature, which for example, can be any protein or polysaccharide or their derivatives. The idea of using the Basonal® X 400 AL binder along with some additional natural polymer (such as starch) in the present invention was that the natural component in the Basonal® binder would promote the compatibility of the additional starch with the Basonal® binder. Compatibility of the different ingredients is important for a barrier coating. To prove the concept, additional tests were run as shown in Table 4 to compare SA binder (PHOPLEX® C-340 from Dow Chemical Company used in the examples) and Basonal® X 400 AL (from BASF Corporation), both including Pen-Cote® D starch in the formulations at a same blend ratio. All of the samples were fully repulpable and non-blocking. As for compostability, as seen in the first three columns of Table 4, paperboard C3 with coating using a styrene acrylate (SA)/Pen-Cote® D binder did not meet the definition of compostability at coat weights of 8-12 pounds. The next three columns show that paperboard CF3 with coating using a Basonal® binder and Pen-Cote® D met the definition of compostability at a coat weight of 8.0 and 9.7 pounds, but not at a high coat weight of 10.8 pounds. Most interestingly, the CF3 (Basonal®+ Pen-Cote® D) coatings had better OGR and moisture vapor

barrier performance, in other words, higher 3M kit and lower Oil Cobb values, lower WVTR values, and approximately equal water Cobb values, compared to the C3 (SA+ Pen-Cote® D) coatings. Tables 3 and 4 thus show that the combined use of Pen-Cote® D specialized starch with Basonal® binder provides improved barrier performance, especially, achieving a 3M kit level of 5+, while meeting the compostability standard, being fully repulpable, and not having blocking problems.

As another way to visualize the test results, the data were plotted as shown in FIGS. 6 and 7. Some of the data on the graphs comes from Tables 3 and 4. Other data are also included. FIG. 6 shows 3M kit level vs. coat weight. The kit value generally increases (improves) as coat weight increases. None of the control samples (using SA binder) were compostable in the coat weight range of 6-12 lbs/3 msf. The samples (CF2 and CF3) using 35 parts of (combined) Basonal® X400AL binder plus Pen-Cote® D starch were compostable except at the highest coat weights (10.2 lbs for CF2 and 10.8 lbs/3 msf for CF3) and gave kit values equal to or better (higher) than the control SA sample at comparable coat weight. Samples using 30 parts of (combined) Basonal® and Pen-Cote® D were all compostable (at least up to at least 11.5 lbs/3 msf), while their kit values tended to be lower than the control and the other samples.

FIG. 7 shows oil Cobb vs. coat weight for the selected samples as in FIG. 6. The oil Cobb generally decreases (improves) as coat weight increases. The compostability (or lack thereof) has already been described. The test samples using (combined) Basonal® and Pen-Cote® D gave oil Cobb tests equal or better (lower) than the test samples using styrene-acrylate binder. Most interestingly, for the samples with a total 30 parts of binder (25 parts Basonal® and 5 parts of Pen-Cote® D), although the 3M kit values were lower than the other formulations with 35 total parts of binder (as FIG. 6), the oil Cobb values were still similar or better than the control sample C1 with 35 parts of pure SA binder. This again proves the synergistic effect of Basonal® with Pen-Cote® D starch.

Some food service or food packaging applications require high quality printing on the external side of the package in addition to a barrier for the food contact side. To demonstrate that a finished paperboard with a barrier coating on one side and a print coating on the other side can meet the composition requirements for the ASTM compostability standard, another experiment was conducted to test print coat formulations that used conventional binders, styrene acrylate (PHOPLEX® C-340 used, available from Dow Chemical Company) and polyvinyl acetate (POLYCO™ 2160 used, available from Dow Chemical Company), with each polymer binder in the coatings meeting the <1% non-biodegradable composition requirement for caliper 12 pt and above, according to the compostability standard ASTM D6868-11. Although the print coat formulations for these tests were adjusted slightly by reducing the content of

## 11

SA binder, the coatings still showed high quality of printability comparable to that of the commercial print grade.

The printable formulations that were tested are summarized in Table 5 for three base coatings and two top coatings described using a basis of 100 parts pigment. Table 6 shows coat weights used in several pilot coater tests for the printable formulations on 18 pt paperboard. Paperboards with the printable test coatings shown in Table 6 all would be compostable according to the ASTM standard, provided the paperboard caliper is 12 pts or higher. This would be true with—or without—the compostable barrier coatings (described above) on the opposite side of the paperboard.

Table 6 also shows the roughness, optical properties, and printability results for the test coatings. Optical properties including Gloss, Brightness, Whiteness, and L-a-b color were measured according to TAPPI standards described above. Parker Print-Surf (PPS) roughness was measured according to TAPPI standard T555. The coated samples were printed on a Harper Phantom QD™ Flexo Proofing System from Harper Corporation using a 2.5 bcm anilox roll with a blue flexo ink. The ink density was measured on an X-Rite 500 series equipment. All test coatings, which would be compostable showed higher gloss, slightly higher brightness, and comparable whiteness over the commercial control. No dyes were used in the test coatings, which in addition to variables in the formulations could contribute to the slight difference of L-a-b color values. All the test coatings showed relatively higher PPS values over the commercial control; however, they were still fairly good, and all of the test coatings after printing showed ink density slightly higher (1.64-1.72 vs. 1.62) than the commercial control, indicating the good printability of the printable test coatings. For the printability tests, a barrier coating was not applied to the opposite side of the paperboard. However, calculations show that the printable paperboard would meet

## 12

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060  
9065  
9070  
9075  
9080  
9085  
9090  
9095  
9100  
9105  
9110  
9115  
9120  
9125

# US 9,863,094 B2

13

TABLE 3

| Effect of Various Binders on Coating Properties including Compostability |             |                 |                                |                                |                                |                                |      |
|--------------------------------------------------------------------------|-------------|-----------------|--------------------------------|--------------------------------|--------------------------------|--------------------------------|------|
|                                                                          | Designation |                 |                                |                                |                                |                                |      |
|                                                                          | C1<br>SA    | C2<br>Basonal ® | CF1<br>Basonal +<br>Pen-cote D | CF2<br>Basonal +<br>Pen-cote D | CF3<br>Basonal +<br>Pen-cote D | CF4<br>Basonal +<br>Pen-cote D |      |
| Coat wt lb/3 msf                                                         | 8.9         | 9.6             | 8.1                            | 9.0                            | 8.4                            | 8.9                            | 9.7  |
| Compostable *                                                            | No          | No              | Yes                            | No                             | Yes                            | Yes                            | Yes  |
| Repulp % accepts                                                         | —           | 100             | —                              | 100                            | 100                            | 100                            | —    |
| 3M kit                                                                   | 2.8         | 5.4             | 3.6                            | 4.6                            | 4.0                            | 5.0                            | 5.2  |
| Oil Cobb                                                                 | 23.7        | 10.2            | 17.5                           | 9.4                            | 11.3                           | 12.3                           | 6.1  |
| grams/(m <sup>2</sup> 30 min)                                            |             |                 |                                |                                |                                |                                |      |
| H <sub>2</sub> O Cobb                                                    | 30.2        | 30.3            | 32.9                           | 32.4                           | 31.2                           | 30.3                           | 29.8 |
| grams/(m <sup>2</sup> 2 min)                                             |             |                 |                                |                                |                                |                                |      |
| WVTR                                                                     | 891         | 764             | 829                            | 758                            | 773                            | 839                            | 790  |
| grams/(m <sup>2</sup> day)                                               |             |                 |                                |                                |                                |                                |      |
| Blocking                                                                 | 1           | 1               | 0                              | 0                              | 0                              | 0                              | 0    |
| Gloss                                                                    | 13.5        | 14.0            | —                              | 13.8                           | —                              | 14.5                           | 16.0 |
| Brightness                                                               | 79.5        | 79.4            | —                              | 76.2                           | —                              | 76.1                           | 75.5 |
| Whiteness                                                                | 66.8        | 66.3            | —                              | 58.2                           | —                              | 57.9                           | 56.3 |
| L-a-b                                                                    | 91.0        | 91.9            | —                              | 91.2                           | —                              | 90.1                           | 90.0 |
| Color                                                                    | 0.4         | 0.4             | —                              | 0.2                            | —                              | 0.2                            | 0.2  |
|                                                                          | 3.4         | 3.5             | —                              | 4.8                            | —                              | 4.9                            | 5.1  |
|                                                                          |             |                 |                                |                                |                                |                                |      |

\* Compostable: defined as less than 1% by weight of non-biodegradable constituent for paperboard calipers of 12 points or higher

25

TABLE 4

| Biodegradability with SA & Basonal ®<br>(Pen-cote ® D added to both) |                         |                                 |      |      |      |      |
|----------------------------------------------------------------------|-------------------------|---------------------------------|------|------|------|------|
|                                                                      | Designation             |                                 |      |      |      |      |
|                                                                      | C3<br>SA + Pen-cote ® D | CF3<br>Basonal ® + Pen-cote ® D |      |      |      |      |
| Coat wt lb/3 msf                                                     | 8.3                     | 10.1                            | 11.6 | 8.0  | 9.7  | 10.8 |
| Compostable                                                          | No                      | No                              | No   | Yes  | Yes  | No   |
| Repulp % accepts                                                     | —                       | 100                             | 100  | —    | 100  | 100  |
| 3M kit                                                               | 1.2                     | 1.8                             | 2.8  | 2.6  | 5.2  | 6.2  |
| Oil Cobb                                                             | 46.5                    | 14.9                            | 6.1  | 45.5 | 6.1  | 2.3  |
| grams/(m <sup>2</sup> 30 min)                                        |                         |                                 |      |      |      |      |
| H <sub>2</sub> O Cobb                                                | —                       | 26.6                            | 28.4 | 31.1 | 29.8 | 31.3 |
| grams/(m <sup>2</sup> 2 min)                                         |                         |                                 |      |      |      |      |
| WVTR                                                                 | —                       | 915                             | 930  | 959  | 790  | 680  |
| grams/(m <sup>2</sup> day)                                           |                         |                                 |      |      |      |      |
| Blocking                                                             | 0                       | 0                               | 0    | 0    | 0    | 0    |

TABLE 5

| Formulations for Printable Coatings |                           |     |     |     |     |     |
|-------------------------------------|---------------------------|-----|-----|-----|-----|-----|
|                                     | Designation               | BC1 | BC2 | BC3 | TC1 | TC2 |
| 30                                  | Clay-1                    |     |     |     | 51  | 30  |
| 35                                  | Clay-2                    |     | 50  |     |     |     |
|                                     | CaCO <sub>3</sub> -1      | 50  | 100 | 100 |     |     |
|                                     | CaCO <sub>3</sub> -2      |     |     |     | 49  | 70  |
| 40                                  | PHOPLEX ® C-340 (SA)      | 19  | 17  | 17  | 4   | 5   |
|                                     | POLYCO ™ 2160 (PVAc)      | 6   | 4   |     | 12  | 11  |
|                                     | Pen-cote ® D UHV (starch) |     |     |     | 4   |     |

TABLE 6

| Printability Tests on Printable Coatings (18 pt<br>paperboard; no barrier coating on opposite side) |                        |                       |         |         |         |         |
|-----------------------------------------------------------------------------------------------------|------------------------|-----------------------|---------|---------|---------|---------|
|                                                                                                     | Designation            | Commercial<br>Control | BC1/TC1 | BC2/TC1 | BC2/TC2 | BC3/TC1 |
|                                                                                                     | BC Coat wt<br>lb/3 msf | 9.4                   | 8.8     | 7.5     | 7.5     | 6.2     |
|                                                                                                     | TC Coat wt<br>lb/3 msf | 4.7                   | 5.4     | 7.2     | 7.1     | 7.1     |
|                                                                                                     | Compostable *          | No                    | Yes     | Yes     | Yes     | Yes     |
|                                                                                                     | Parker PrintSurf       | 1.47                  | 1.50    | 1.80    | 1.94    | 1.82    |
|                                                                                                     | Gloss                  | 46.6                  | 56.4    | 57.1    | 52.2    | 57.5    |
|                                                                                                     | Brightness             | 83.5                  | 84.6    | 84.9    | 85.5    | 85.0    |
|                                                                                                     | Whiteness              | 77.4                  | 75.9    | 77.0    | 78.6    | 77.3    |
|                                                                                                     | L-a-b                  | 92.0                  | 93.2    | 93.2    | 93.3    | 93.2    |
|                                                                                                     | Color                  | -0.4                  | 0.4     | 0.5     | 0.5     | 0.4     |
|                                                                                                     |                        | 1.6                   | 2.4     | 2.2     | 1.8     | 2.1     |
|                                                                                                     | Ink Density            | 1.62                  | 1.64    | 1.71    | 1.72    | 1.71    |

(\* Compostable: defined as less than 1% by weight of non-biodegradable constituent for paperboard calipers of 12 points or higher)

## 15

The invention claimed is:

1. A coated paperboard comprising:  
a paperboard substrate having a first side and a second side;  
a first coating in contact with the first side, the first coating having a coat weight from 5 to 12 lbs per 3000 ft<sup>2</sup> and comprising binder and pigment, the first coating containing substantially no fluorochemical or wax;  
a second coating in contact with the second side, wherein the second coating is a printable coating;  
wherein the coated paperboard has a caliper of at least 0.010";  
wherein the coated paperboard provides barrier properties to at least one of oil, grease, and moisture;  
wherein the coated paperboard is compostable according to the ASTM D6868-11 standard for compostability; and  
wherein the coated paperboard is at least 99% repulpable.
2. The coated paperboard of claim 1, wherein the coated paperboard has a caliper of at least 0.012".
3. The coated paperboard of claim 1, wherein the binder to pigment ratio in the coating is between 25 to 40 parts binder per 100 parts pigment, by weight.
4. The coated paperboard of claim 3, wherein the binder to pigment ratio in the coating is between 30 to 35 parts binder per 100 parts pigment, by weight.
5. The coated paperboard of claim 1, wherein the binder comprises a synthetic polymer including (i) a non-biodegradable component and (ii) a natural biodegradable component.
6. The coated paperboard of claim 5, wherein the binder further comprises (iii) an additional natural biodegradable component.
7. The coated paperboard of claim 6, wherein the additional biodegradable component (iii) is at least one of polysaccharide and protein.
8. The coated paperboard of claim 6, wherein the additional biodegradable component (iii) comprises between 1 to 7 parts starch per 100 parts pigment, by weight.
9. The coated paperboard of claim 1, wherein the 3M kit test value is at least 3.
10. The coated paperboard of claim 1, wherein the coated paperboard has a 30-minute oil Cobb test of at most 20 grams per square meter.
11. The coated paperboard of claim 1, wherein the coated paperboard is repulpable to the extent that after repulping the percentage accepts is at least 99%.

## 16

12. The coated paperboard of claim 11, wherein the percentage accepts is at least 99.9%.
13. The coated paperboard of claim 1, wherein the coating weight is 5 to 12 lbs per 3000 ft<sup>2</sup>.
14. The coated paperboard of claim 13, wherein the coating is applied in two passes for a total coat weight of 5 to 12 lbs per 3000 ft<sup>2</sup>.
15. The coated paperboard of claim 1, having no tendency toward blocking after being held for 24 hours at 50° C. at a pressure of 100 psi.
16. The coated paperboard of claim 1, wherein the pigment comprises at least one of a clay and calcium carbonate.
17. A method of treating paperboard, the method comprising:  
providing a paperboard substrate having a first side and a second side;  
applying to the first side a coating comprising binder and pigment, and containing substantially no fluorochemical or wax;  
applying to the second side a printable coating;  
wherein the binder comprises starch;  
wherein the treated paperboard has a caliper of at least 0.010";  
wherein the treated paperboard is compostable according to the ASTM D6868-11 standard for compostability;  
wherein the treated paperboard has a 3M kit test value of at least 3; and  
wherein the treated paperboard is repulpable to the extent that after repulping the percentage accepts is at least 99%.
18. The method of claim 17, wherein the coating is applied by a device selected from the group consisting of a blade coater, curtain coater, air knife coater, rod coater, film coater, short-dwell coater, spray coater, and metering film size press.
19. A coated paperboard comprising:  
a paperboard substrate;  
a base coating in contact with the paperboard substrate, the base coating having a coat weight from 6 to 10 lbs per 3000 ft<sup>2</sup> and comprising binder and pigment;  
a top coating in contact with the base coating, the top coating having a coat weight from 4 to 7 lbs per 3000 ft<sup>2</sup> and comprising binder and pigment;  
wherein the coated paperboard has a caliper of at least 0.010"; and  
wherein the coated paperboard is compostable according to the ASTM D6868-11 standard for compostability.

\* \* \* \* \*